

## UNITED STATES PATENT OFFICE

2,343,956

## DEEP HARDENING SILICON TITANIUM STEEL

Walter Crafts, Niagara Falls, N. Y., assignor to  
Electro Metallurgical Company, a corporation  
of West Virginia

No Drawing. Application June 30, 1942,  
Serial No. 449,163

## 4 Claims. (CL 75—123)

This invention relates to steels, and more specifically to steels the hardness of which may be increased by rapid cooling from temperatures within or above the critical range. This application is a continuation-in-part of my copending application, Serial No. 321,915, filed March 2, 1940. The invention will be described herein as it may be applied to carbon steels containing between 0.2% and 1% carbon, up to about 2% manganese, between 0.50% and 2% silicon and between 0.05% and 0.15% titanium.

When hardening steels by rapid cooling from high temperatures, it is often desired to produce a deep or thick zone of hardened material rather than a thin or shallow hardened case. The depth to which a piece of steel will harden, at a given rate of heat extraction, is different in different steels. The property of the steel which involves this relative susceptibility to mass effect in hardening seems to be inherent, and for convenience it will be termed herein "deep-hardenability."

An accepted, convenient measure of deep-hardenability is afforded by the "Jominy" test, described in detail in "A Hardenability Test for Carburizing Steel" by W. E. Jominy and A. L. Boegehold, Trans. Am. Soc. for Metals, vol. 26, p. 574 (1938). To summarize briefly, the test is made on a small bar of steel of standardized shape and dimensions, and comprises heating the entire bar to the desired hardening temperature, quickly extracting heat through one end face of the bar, grinding off superficial scale and decarburized skin and producing a flat surface suitable for a hardness test, and measuring the Rockwell C hardness along the length of the bar. The distance from the hardened end at which the hardness becomes less than Rockwell C 50 is referred to herein as the "Jominy depth." If the same hardening temperature and cooling conditions be used for a series of steels, the relative depths of the hardened zones indicate the relative deep-hardenability of the steels of that series, each to the others.

An object of this invention is to improve the deep hardenability of hardenable steels generally, and of plain carbon and low-alloy steels (less than 5% in the aggregate of steel-strengthening elements, for example, chromium, tungsten, molybdenum and nickel) especially.

A further object of this invention is to provide deep-hardenable steels of novel compositions, and deep-hardenable articles made therefrom.

The deep-hardenability of steel may be enhanced in some degree by adding in suitable percentages any one of the elements which can be taken into solid solution in steel at high temperatures, for instance, boron, silicon, molybdenum, tungsten, chromium, or nickel. These hardening elements differ widely in the minimum percentage required to impart a useful degree of

deep-hardenability, and in the maximum degree of deep-hardenability obtainable while maintaining other necessary properties of the steel.

I have observed that combinations of certain elements may be used to impart a greatly enhanced deep-hardenability without substantial sacrifice of other desirable properties of the steel. The present invention is based on these observations.

More specifically, the invention comprises the addition to a hardenable silicon steel of the special element titanium in a suitable percentage greater than that required for grain refinement. The silicon content of the steel of the invention is between 0.50% and 2%. The titanium content of the steel is between 0.05% and 0.15%.

When the above-described percentages of silicon and titanium are employed, a medium manganese oil hardening type of steel such as the S. A. E. 1345 type may be hardened to 50 Rockwell C or higher throughout a circular section one inch, or even more, in diameter.

There appear to be optimum percentages of silicon and titanium which impart a maximum depth of hardenability and a frequent result of an increase in percentage beyond the optimum is a decrease of deep-hardenability below that imparted by the optimum. For reasons of economy, or to obtain a steel having a certain desired combination of physical properties, it will often be desired to add either less or more of the elements than will impart a maximum depth of hardening. Hence, the invention is not limited to the use of the optimum percentages.

It has also been found advantageous to add at least one of the elements calcium, barium and strontium in a total percentage between 0.03% and 0.50%.

Typical effects of representative combinations used according to this invention are indicated in Table A, which contains figures derived from actual test data. The relative Jominy hardenability depths are given, in hundredths of an inch, of steels containing besides iron the percentage of silicon and special elements indicated. The same hardening temperature and cooling conditions were used in all tests.

Table A

| Composition of steels:<br>about 1.0% Mn,<br>0.45% to 0.55% C,<br>Si and Ti as indicated,<br>rest Fe |        | Jominy hardness test,<br>depth in hundredths of<br>an inch to Rockwell C<br>50, corrected to 0.45% C<br>by factor: $\pm 0.01\% C =$<br>$\pm 0.012$ inch |
|-----------------------------------------------------------------------------------------------------|--------|---------------------------------------------------------------------------------------------------------------------------------------------------------|
| % Si                                                                                                | % Ti   |                                                                                                                                                         |
| 1 0.50                                                                                              | 1 0.12 | 33                                                                                                                                                      |
| 0.77                                                                                                | 0.12   | 80                                                                                                                                                      |
| 0.95                                                                                                | 0.13   | 115                                                                                                                                                     |

<sup>1</sup> Nominal.

The high quality attainable in steels according to this invention is indicated in Table B by test data of the physical properties of two representative steels after forging, quenching from 850° C., and drawing at 400° C. for one hour. In Table B, the yield point (Y. P.) and tensile strength (T. S.) of the steels are given in thousands of pounds per square inch; El. designates percentage elongation in a two inch initial gauge length, and %R. A. designates percentage reduction of area upon fracture of the 0.505 inch diameter standard (A. S. T. M.) tensile test specimens. Under "Izod" are given the Izod impact test results, in foot pounds, using a standard specimen one-centimeter square with standard V notch two mm. deep. The Jominy hardness test depth is that actually measured, in hundredths of an inch, to Rockwell C 50, the same hardening temperature and cooling conditions having been used in all hardness tests. The steels contain about 1.7% manganese, about 0.50% carbon, silicon and titanium as indicated, rest iron.

Table B

| Composition |      | Physical |       | Properties of steels |         |      |                            |
|-------------|------|----------|-------|----------------------|---------|------|----------------------------|
| % Si        | % Ti | Y. P.    | T. S. | % El.                | % R. A. | Izod | Jominy hardness test depth |
| 0.77        | 0.12 | 199.0    | 220.5 | 11.0                 | 38.2    | 8.7  | 87                         |
| 0.95        | 0.13 | 218.0    | 238.5 | 8.5                  | 39.8    | 7.5  | 116                        |

The advantages of the invention may be exploited in any of several ways. For instance cheaper steels may be used instead of more expensive, more highly alloyed steels heretofore used to obtain the desired strength. Or, present high strength steels may be even further strengthened by applying the principles of the invention, either by deeper hardening to a lower average hardness or by deeper hardening to the

same or even higher hardness. Among the various steels described, there is a wide range of choice in respect to such factors as cost, grain size control, ductility, strength, and toughness. 5. Thus, the invention is capable of a wide field of application, which will be apparent to metallurgists and steel makers. Therefore, although specific examples have been given herein to illustrate the principles of the invention, it will be 10 understood that such examples are merely illustrative and do not restrict the invention beyond the requirements of the claims and the state of the art.

I claim:

15. 1. A hardenable steel which is hardenable to at least 50 Rockwell C throughout a one inch diameter circular section, comprising substantially more than 0.5% up to 2% silicon; between 0.2% and 1% carbon; manganese in a percentage up to about 2%; titanium between 0.05% and 0.15%; remainder substantially all iron.

2. A hardenable steel as defined in claim 1, also containing at least one of the alkaline earth metals calcium, barium, and strontium, the total 25 addition of such alkaline earth metals being between 0.03% and 0.50%.

3. A quench-hardened article composed of a deep-hardenable steel comprising substantially more than 0.5% up to 2% silicon; between 0.2% and 1% carbon; manganese in a percentage up to about 2%; titanium between 0.05% and 0.15%; remainder substantially all iron, such 30 steel having the property of being quench-hardenable to upwards of 50 Rockwell C throughout a one inch diameter circular section.

4. A quench-hardened article composed of a deep-hardenable steel as claimed in claim 3, also containing at least one of the alkaline earth metals calcium, barium, and strontium, the total 40 addition of such alkaline earth metals being between 0.03% and 0.50%.

WALTER CRAFTS.